

Oct. 24, 1933.

W. D. NICOLL

1,931,933

MANUFACTURE OF HIGH ALPHA CELLULOSE PULP

Filed Jan. 6, 1933

3 Sheets-Sheet 1



Fig. 1

INVENTOR.

William D. Nicoll  
BY Ralph F. Miller

ATTORNEY.

Oct. 24, 1933.

W. D. NICOLL

1,931,933

## MANUFACTURE OF HIGH ALPHA CELLULOSE PULP

Filed Jan. 6, 1933

3 Sheets-Sheet 2



Fig. 2



Fig. 3

*INVENTOR.*

BY William D. Nicoll  
BY Ralph F. Miller

*ATTORNEY.*

Oct. 24, 1933.

W. D. NICOLL

1,931,933

## MANUFACTURE OF HIGH ALPHA CELLULOSE PULP

Filed Jan. 6, 1933 3 Sheets-Sheet 3

## DIGESTERS

Nº1 Nº2 Nº3 Nº4



## CYCLE OF OPERATION FOR EACH DIGESTER IN ONE BANK OF FOUR DIGESTERS

Fig. 4

*INVENTOR.*

William D. Nicoll  
BY Ralph F. Miller

*ATTORNEY.*

## UNITED STATES PATENT OFFICE

1,931,933

MANUFACTURE OF HIGH ALPHA  
CELLULOSE PULP

William D. Nicoll, Wilmington, Del., assignor to  
E. I. du Pont de Nemours & Company, Wil-  
mington, Del., a corporation of Delaware

Application January 6, 1933. Serial No. 650,551

9 Claims. (Cl. 92—13)

This invention relates to the manufacture of paper pulp, and more particularly to the production of a pulp characterized by a high alpha cellulose content and adapted for use in the manufacture of rayon, cellophane, and various derivatives of cellulose.

This invention has as an object the preparation of a high alpha pulp from raw cellulose material by a process involving a single digestion with alkaline solutions. A further object is to provide an improved process which is peculiarly adapted for the successful and economical manufacture of high alpha cellulose pulp from the structural fibers of plants of the grass family (Gramineæ) and in particular to provide a means of producing high alpha cellulose from the fiber of pith bearing plants of the grass family such as sugar cane or corn. Other objects will appear hereinafter.

These objects, in accordance with my preferred practice using sugar cane bagasse, are accomplished by the following process in which bagasse is first very thoroughly depithed and then treated in digesters under pressure and at temperatures above 100° C. with cooking liquors which are made to flow in such a manner that the fiber is treated with liquors containing progressively increasing concentrations of active cooking agent and decreasing concentrations of dissolved organic material. The crude pulp produced in this manner is washed free of cooking liquors, screened to remove shives (incompletely digested fibers), and bleached by means of a two stage process involving first a treatment with chlorine water and then with hypochlorite. At the end of the bleaching process the pulp is washed with an acid solution and then with pure water.

The method for carrying out my invention is illustrated by the accompanying drawings in which

Fig. 1 is a flow sheet of the complete process; Figs. 2 and 3 illustrate the digestion procedure and circulation of liquor; and Fig. 4 is a schematic drawing showing the complete cycle of operation for each digester in a bank of four digesters.

Having reference to Fig. 1, which is a flow sheet of the complete process, the bagasse, after shredding and screening, is thoroughly depithed. This depithing or separation of the long structural fibers from the small pith cells characteristic of mill run bagasse is efficiently effected by passing the material through an attrition mill or any apparatus giving similar mechanical treatment

and then screening out the pith to permit the satisfactory circulation of caustic liquors through the pulp. It is important to the successful operation of the present process that the bagasse be very thoroughly depithed. The depithing is, therefore, carried out to an extent which removes from 35% to 40% of the weight of the bagasse undergoing the depithing operation. In this manner, in most cases, more than 90% of the total amount of pith originally present is removed. Since the pith screenings may contain more or less of the fiber and since the original proportion of pith to fiber varies somewhat the optimum proportion to be separated as pith is also variable, the essential requirement being that enough pith be separated so as to permit circulation of the caustic liquor under moderate pressure. This substantially complete removal of the pith may be effected by a preliminary rough screening of the bagasse as received from the mill to remove a portion of the pith; passing of the screened fiber through the attrition mill to loosen the adhering pith cells; final screening of the fiber and pith from the attrition mill in order to thoroughly separate the fiber from the pith, with the result that the fiber only is passed to the digesters. Another satisfactory procedure consists in passing all of the mill run bagasse directly to the attrition mill from which it is passed over screens for the thorough removal of the pith, the resultant clean fiber going direct to the digesters.

The next or digestion step, which is one of the principal features of the present process, will be described in detail below. The remaining steps indicated on the diagram will be well understood by those skilled in the art of paper making. With reference to refining and bleaching, the crude pulp may be refined in any known manner as, for instance, by first screening and riffling the crude stock to remove such particles or undigested fiber as may remain in the pulp and to settle out heavy ash particles which cannot be removed by chemical means. To facilitate the screening and washing of the pulp and to remove liquor and ash, water may be vigorously sprayed on the pulp as it passes over a series of drum screens or washers. The washed pulp is then partially bleached by treatment first with chlorine while violently agitated in a tank. The amount of chlorine used is less than that required for complete reaction with the pulp but sufficient to react with a large part of the lignin, pentosans, etc. The chlorinated pulp is then washed with a dilute solution of caustic soda in order to dis-

solve chlorinated organic compounds. After this the partially bleached pulp is treated with calcium or sodium hypochlorite in sufficient amount to produce a white color in the pulp. If desired, 5 the stock may be acidified before removing the final bleach liquor or it may be given a separate acid treatment after the bleach is removed. After washing with pure water and drying, the pulp is ready for use. The total chlorine consumed on a typical pulp may be 2.5% of the weight of the pulp of which 60% may be used as free chlorine in the first stage of bleaching and 40% as calcium hypochlorite in the second stage of bleaching.

10 Before bleaching, the amount of chlorine necessary to produce a satisfactory white pulp is determined by any one of several known tests used in the industry for this purpose. This chlorine is applied in two stages. The preferred process 15 involves treating the pulp at 3% consistency with free chlorine water to the extent of 60% of the necessary chlorine and after exhaustion of this chlorine treating the pulp with just sufficient alkali to produce an alkaline reaction. Treatment 20 with alkali dissolves any chlorinated lignin compounds from the cellulose and these soluble compounds are washed away by water. Following this, the second stage of bleaching is carried out by treating the pulp at a 10% consistency with the 25 remaining 40% of necessary chlorine in the form of calcium hypochlorite until a white color is produced. The pulp slurry is acidified at the end of the bleach and washed free of chlorine and acid. The bleached pulp is then ready to form 30 35 into board, paper, etc.

Before proceeding with the description of the method of digestion used in the present process, it may be noted that a pretreatment with water is, in some instances, desirable. In the digestion 40 step of the process an optional water digestion may precede the regular digestion by treating the fiber with hot water between 100-200° C., and preferably between 130-160° C., under pressure. At the end of this treatment the water 45 may be conveniently blown from the digester and the digestion continued with alkali in the manner outlined below.

As an illustration of the pretreatment with water before regular digestion with caustic solution 50 the depithed bagasse is charged into a digester and treated for one hour with hot water at 150° C. Such a treatment will dissolve from 10-20% of the original bagasse as water-soluble compounds, and these may be removed from the fiber by blowing out the water as completely as possible at the end of the treatment. Fiber which is thereby reduced to between 80 to 90% of its original weight is subsequently countercurrently digested with the caustic solutions.

60 One method of carrying out the digestion process will be described as it can be applied in a battery of four digesters. It is assumed that the process is in full operation and that the cycle of operations which is described as occurring in 65 a system of four digesters is equally applicable to each separately in proper sequence. The digestion process can perhaps be most easily described if it is considered as made up of six separate cooks which may be taken as periods during which each 70 digester is isolated and the cooking liquors circulated through outside heaters to maintain temperatures. The strength of the caustic soda increases and the amount of dissolved organic matter decreases as the cooking progresses from 75 cooks 1 to 6 so that the cooking under the pre-

ferred practice of the invention is, therefore, semi-countercurrent in nature. In Figs. 2 and 80 3 are shown diagrammatic views of the digestion process during the two principal liquor transfer operations which occur alternately between the progressive stages of digestion. It will be understood that the system of piping has been greatly simplified so that only the bare essentials required to indicate the transference of cooking liquors are shown. The quantities of liquor indicated as transferred in any one operation are merely representative of the general cooking procedure and so are conveniently taken as fractions of the full capacity of one digester. During operation the various digesters are always maintained nearly full for circulation is, in most cases, 90 in an upward direction through the digesters.

Starting with the system as represented in Fig. 2, it will be seen that cooking is taking place in digesters 1, 2 and 3 while No. 4 is out of service and is being filled with a fresh charge of fiber. It may be well to state here that during the charging of any digester a certain amount of spent liquor is sprayed in with the fiber to help wilt it so that a maximum charge may be used; this is made 100 necessary by the fact that the fibers do not otherwise pack readily. As far as the other three digesters are concerned, it will be assumed that cooking has progressed so that No. 1 digester has just completed its fifth cook and is ready for its 105 sixth and last cook, No. 2 digester has just completed its third cook or is ready to start its fourth cook, and No. 3 digester has just completed its first cook and is therefore starting its second cook.

110 The liquor transfer represented in Fig. 2 consists in introducing fresh strong caustic through the system at A, pumping it by means of pump 10 through the valved conduit 11, 12 and 13 into the bottom of No. 1 digester and so displacing from the top of this digester practically all the liquor which it contains. The liquor leaving the top of No. 1 digester through pipe 14 surrounded by heater H is forced, by means of the pump 15 located under No. 1 digester, into the bottom of No. 2 digester through the valved conduit 16 and 17 as indicated by the arrows. The liquor in No. 2 digester is, in similar manner, displaced into No. 3 digester and the nearly spent liquor in No. 3 digester is forced out of the digestion system at B. 125 The amount of liquor displaced through the system in this transfer is approximately equal to a full digester charge so that at the end of the transfer the change of liquor has been practically complete in every digester involved. The three digesters Nos. 1, 2 and 3 are then isolated and the liquor allowed to circulate through the outside heaters in each case. The temperature of the cooking liquors is maintained at the proper level during both the transfer of liquor from one digester to another and during the period of isolation by the continual passing of said liquors through the heaters H.

130 A part (in this case 2/3) of the nearly spent liquor taken from the system at B during the foregoing transfer is held in storage for a short time and then as already noted is returned to the digestion system to help wilt the fiber during the filling of another digester. The remainder of the spent liquor is sent to the recovery system for the 135 regeneration of fresh cooking liquor.

140 Following the period during which each digester is operated independently the next transfer of liquor is represented by Fig. 3 in which digesters Nos. 1, 2 and 3 have just completed their sixth, fourth 150

and second cooks, respectively. Digester No. 1 is, therefore, ready to be taken out of service and digester No. 4 is to start on its first cook. During this transfer fresh caustic is not introduced into the system but the liquor to be displaced through the system is drawn from the bottom of No. 1 digester. The amount of liquor transferred is also much less in this case than in the first transfer, for only about one-third of a digester charge is so displaced. Digester No. 4 (going into service) is already filled to approximately two-thirds its capacity with nearly spent liquor which was added during the charging of the digester, and the displacement of liquor from the rest of the system is stopped as soon as No. 4 digester is filled. As soon as this is done each digester is again isolated and circulation started in digesters Nos. 2, 3 and 4.

The completion of the foregoing transfer leaves digester No. 1 approximately two-thirds filled with fairly strong cooking liquor and completely cooked pulp. The strong liquor is blown out through the false bottom of the digester into a storage tank from which it is returned to the digestion system after fortifying as fresh cooking liquor. The crude pulp in digester No. 1 is washed once with hot water in the digester, and then blown from the digester along with the second wash water, and is thereafter ready for the refining and bleaching operations. The empty digester No. 1 is refilled with fiber in the same manner as already described for digester No. 4. At the end of the circulation period in progress, fresh cooking liquor is introduced into No. 2 digester in order to force a complete displacement of liquor through Nos. 2, 3 and 4 digesters in exactly the same manner as the first transfer already described for Nos. 1, 2 and 3 digesters. The whole cooking cycle has moved forward one digester, thus completing the cycle of operation so far as the system as a whole is concerned.

It will thus be seen that the system illustrated in Figs. 2 and 3 has four digesters, in each of which the cooking is continued from an initial to a final cook, the stage of cooking also progressively increasing from an initial cook in the digester at one end of the system to a final cook in the digester at the other end. In Fig. 3 the initial cook is beginning in digester No. 4 and the final cook has ended in digester No. 1, from which the purified pulp is blown. The liquor in circulation with the other digester is cut off and the empty digester, which is now No. 4 in Fig. 2, is charged with bagasse. The liquor of the remaining digesters, now designated as Nos. 2, 3 and 4 in Fig. 3, is then displaced from one digester to another, the spent liquor from digester No. 4 of Fig. 3 which contains the first cook being introduced with the new charge of bagasse as described above.

In Fig. 4 is shown a schematic arrangement of the complete cycle of operation for each digester in one bank of four digesters. The method for operating the process as referred to above is depicted. A complete cycle of operation for each digester in one bank of four digesters is shown. In this figure the horizontal circles represent the static stages described in the detailed description above, and each perpendicular row of circles represents all the various stages (static) of digestion as carried out in the individual digester whose number is given at the top. The numbers in the circles indicate the various stages of digestion; number 1, for example, being the first stage in the cooking of the raw fiber, while number 6 is the last stage of digestion just prior to

washing and discharging the finished pulp. The letter W represents the stages in which the pulp is washed in the digesters and the letter F the periods during which the digesters are filled with raw fiber. The spaces between the horizontal rows of circles represent periods during which transfers of liquors take place and the arrows indicate the direction of flow of the liquors between individual digesters. The fractional numbers accompanying the arrows in this figure as well as in Figs. 2 and 3 indicate the amounts of liquor transferred in any one dynamic stage of digestion, for example,  $3/3$  indicates a complete change of liquor in each digester. The notations at the side of the block of circles deal with the input and output of the various materials which are either used in or are products of the digestion process.

My improved process is best carried out with caustic concentrations between 6% and 9%. Concentrations between 6% and 12% may, however, be used satisfactorily, but the process becomes less economical when the concentration rises above 9%. It will be understood that these concentrations refer not only to sodium hydroxide but also to equivalent strengths of other cooking liquors such as a mixture of sodium hydroxide and sodium sulfide. Thus I may use with satisfactory results a kraft type digestion liquor in which the alkalinity is obtained by using about two-thirds sodium hydroxide and one-third sodium sulfide. I prefer to operate at a temperature of about 140° C. Deterioration sets in too rapidly at temperatures above 160° C., and below 130° C. the time required is too long, the efficiency reduced, and difficulty is encountered in removing the last of the non-alpha cellulose material. The maximum pressures obtained during the digestion process are dependent on the temperature and concentration of the dissolved matter in the liquors and to some extent on the presence of any gases formed during digestion. For example, at a cooking temperature of 140° C., the pressure in the digesters will be about 50 pounds. These gases may be relieved from the digesters from time to time. The total time during which a single batch of fiber is undergoing digestion will depend on the concentration of alkali used, the temperature, and the pressure at which the digestion is carried on. Roughly, the time of digestion is inversely proportional to the product of these factors. With respect to time, it may be stated generally, therefore, that the process is continued until a high alpha cellulose is obtained, i. e., a pulp containing not less than about 95% alpha cellulose. A convenient time for a complete cook is 7 hours operating at a temperature of 140° C. and a pressure of 50 pounds per square inch.

Since the grinding season in the sugar countries does not extend over the entire year, it is necessary to store some of the depithed fiber. This may be conveniently done either baled or loose, but under cover so as to be out of the weather. The stored fiber may be drawn on as needed by the digesters.

The digestion process as outlined above gives only one example of several possible variations of the procedure for carrying out a semi-continuous countercurrent digestion of bagasse and, therefore, must not be understood as limiting the scope of my invention. For example, the process may be altered to decrease the amount of liquor displaced during the transfer in which fresh caustic is introduced so that a complete change of liquor

is not obtained and only the quantity of spent liquor which is to be sent to recovery is removed from the digestion system. If this is done the alternating transfer, or that in which liquor is drawn from the completely cooked pulp, becomes greater so that a nearly complete displacement of liquor throughout the system is obtained. By still other procedures the two principal liquor transfers may be made almost equal in amount or they may conform to any desired amount between the two extremes represented by the first and second procedures.

With reference to the procedure described in connection with Figs. 2 and 3, it will be apparent that the amount of liquor transferred through the system when a new digester is put into service is relatively small when compared to the amount of liquor transferred when fresh caustic is added to and waste liquor removed from the system. The following is an example of the procedure outlined above with the exception that the amounts of liquor transferred at any one time are different. The weights of materials given refer to operation in a battery of four small digesters used in the development of the digestion process on a small scale in which the total liquor capacity of each digester is about 525 pounds of water.

The charge of fiber is 45-50 pounds of depithed bagasse containing about 25% moisture and the yield of high alpha pulp approximately 15 pounds or 40%, based on the dry fiber charge. Fresh caustic solutions added to the system contain alkali (sodium hydroxide and sodium carbonate) equivalent in sodium content to a 9% sodium hydroxide solution which produces a cooking liquor equivalent to an 8% caustic solution. For a given initial caustic concentration the amount of free caustic in the waste may be controlled within limits by varying the total amount of liquor passing over the fiber. Thus when the initial concentration is around 8% sodium hydroxide, the free caustic in the waste black liquor may readily be reduced to 1% or even below by limiting the amount of liquor drawn off at each stage. Under this system of operation each time fresh caustic is introduced into the system 450 pounds is the amount added, and 400 pounds of black liquor is removed at the opposite end of the system. One hundred pounds of this black liquor is sent to waste and 300 pounds returned to the next freshly charged digester. The cycle is completed by recovering alkali from the black liquor in known manner, including the steps of concentrating the liquor, burning the organic matter, causticizing and using the recovered caustic in the digesters. When a new digester is put into service the amount of liquor displaced through the system is small since only about 150 pounds of strong liquor need to be pumped from digester No. 4 through digesters Nos. 3 and 2 to completely fill No. 1 digester. During the periods between liquor transfers, each digester is isolated as previously described and the liquors circulate in each through the outside circulation pipe. The completion of the foregoing transfer leaves digester No. 1 approximately two-thirds filled, i. e., about 350 pounds, with fairly strong cooking liquor and completely cooked pulp. The strong liquor is blown out through the false bottom of the digester into a storage tank from which it is returned to the digestion system. The time required for the transfer in which the caustic is introduced is about 30-45 minutes and for the transfer involving the starting of a new digester is be-

tween 15 to 30 minutes. The total digestion time is about 7½ hours with each charge started one and one-quarter hours apart. The pulp produced by the foregoing process averages 95-96% alpha cellulose.

Another variation in digestion procedure is to eliminate entirely the periods during which each digester is isolated and the liquor circulated separately in each. Carrying out this modification the transfer of liquors is slowed down so that the time of transfer and isolation is all taken up by the transfer only. Under these conditions digestion proceeds as usual and the temperature is maintained by the flow of liquor through the heaters during the transfer.

The present process may utilize raw cellulose material from plants of the grass family such as bamboo, brava cane, sugar cane, esparto, and corn stalks, and is particularly advantageous when applied to the preparation of high alpha pulp from pith bearing plants such as corn and sugar cane.

An important advantage of this process over known methods of preparing high alpha pulp from vegetable materials is to be found in the fact that the crude fiber is converted in one step whereas other known processes for treating raw gramineous fiber involve two or more separate treatments, such as an acid and alkaline treatment or two distinct alkaline treatments, one usually with a very concentrated alkaline solution. The advantages of processing bagasse and similar pith bearing fibers for the production of high alpha cellulose by the countercurrent treatment under pressure as described herein, has not, insofar as I am aware, been disclosed. An important finding which has made possible the successful production of high alpha cellulose from bagasse (the term "bagasse" being used to designate also raw cellulose material of like nature) by the one step process described above is the discovery of the marked advantage which results when the pith is so thoroughly removed from the fiber that substantially none remains. While the depithing of bagasse is in itself not new, it is to be observed that it has not previously been used with countercurrent digestion under pressure, and that my process is characterized by removal of the pith from the fiber to an extent beyond that heretofore practiced or necessary in prior processes, and that the fiber thus prepared is converted in one cook to a high alpha cellulose pulp by the continuous countercurrent process described. In the present pressure digestion process any appreciable pith content of the fiber prevents adequate circulation of the cooking liquors, it being practically impossible to circulate the caustic liquors and, therefore, impossible to carry out the present countercurrent process unless the pith is first substantially removed. Furthermore, I find that the thorough removal of the pith from bagasse decreases the consumption of caustic and markedly improves the quality of the product for such uses as rayon, cellophane and cellulose derivatives.

An additional advantage of my invention resides in the fact that high alpha cellulose is obtained by a process in which nearly all the caustic is used. This result is brought about by controlling the flow of digestion liquor so that the waste liquor is practically stripped of free caustic. Another advantage resides in the fact that the liquors contain enough organic

80

85

90

95

110

115

120

125

130

135

140

145

matter to enable the caustic to be burned in recovering the caustic.

As many apparently widely different embodiments of this invention may be made without departing from the spirit and scope thereof, it is to be understood that I do not limit myself to the specific embodiments thereof except as defined in the following claims.

I claim:

10. 1. A process of producing high alpha cellulose pulp which comprises countercurrently digesting raw gramineous fiber substantially free from pith in alkaline liquor maintained at 130-160° C., and washing the pulp, said countercurrent digestion being continued until a pulp is obtained which contains not less than about 95% alpha cellulose on the dry basis.

15. 2. The process set forth in claim 1 in which the alkaline liquor is of 6 to 12% concentration expressed in terms of sodium hydroxide.

20. 3. A process of manufacturing purified cellulose pulp which comprises removing substantially all of the pith from a pith bearing plant of the grass family, countercurrently digesting the raw 25 depithed fiber with alkaline liquor at elevated temperature and pressure, and washing the pulp.

25. 4. A process of producing high alpha cellulose pulp which comprises removing at least 35% of the weight of sugar cane bagasse in the form of 30 pithy material, countercurrently digesting the depithed bagasse in alkaline liquor of 6% to 12% initial concentration expressed in terms of sodium hydroxide, said liquor being maintained at 130-160° C., and washing the pulp, said countercurrent digestion being continued until a pulp is obtained which contains not less than about 95% alpha cellulose on the dry basis.

35. 5. A process of manufacturing purified cellulose pulp which comprises depithing a pith bearing plant of the grass family, countercurrently digesting the raw depithed fiber with caustic liquor, washing the pulp, sufficient pith being separated in the depithing so that the caustic liquor may be circulated under moderate pressure.

6. A process of producing high alpha cellulose pulp which comprises countercurrently digesting raw gramineous fiber substantially free from pith in alkaline liquor maintained at 130-160° C., and washing the pulp, said countercurrent digestion being continued until a pulp is obtained which contains not less than about 95% alpha cellulose on the dry basis, the digestion of the raw fiber being a multiple stage countercurrent digestion in an extraction system which includes at least three digesters through which the liquor passes in series.

80. 7. A process of producing high alpha cellulose pulp which comprises countercurrently digesting raw gramineous fiber substantially free from pith in alkaline liquor maintained at 130-160° C., and washing the pulp, said countercurrent digestion being continued until a pulp is obtained which contains not less than about 95% alpha cellulose on the dry basis, the digestion of the raw fiber being a multiple stage countercurrent digestion in which the liquor passes in series.

85. 8. A process of producing high alpha cellulose pulp which comprises removing at least 35% of the weight of sugar cane bagasse in the form of 90 pithy material, digesting the depithed bagasse with hot water and then countercurrently digesting the treated bagasse in alkaline liquor maintained at 130-160° C., and washing the pulp, said countercurrent digestion being continued until a pulp is obtained which contains not less than about 95% alpha cellulose on the dry basis.

95. 9. A process of producing high alpha cellulose pulp which comprises countercurrently digesting raw gramineous fiber substantially free from pith 100 in alkaline liquor maintained at 130-160° C., and washing the pulp, said countercurrent digestion being continued until a pulp is obtained which contains not less than about 95% alpha cellulose on the dry basis, and subjecting the 105 treated pulp to a partial bleach followed by a final complete bleach.

WILLIAM D. NICOLL.

120

125

130

135

140

145

150

50

55

60

65

70

75